

## UNITED STATES PATENT OFFICE

1,981,514

PROCESS FOR THE PRODUCTION OF  
PRESS-MOLDING MASSES BY CONDENSA-  
TION OF PHENOLS WITH FORMALDE-  
HYDE OR SUBSTANCES THAT YIELD  
FORMALDEHYDE

Max Koebner, Ludwigshafen-on-the-Rhine, Germany, assignor to F. Raschig G. m. b. H., Ludwigshafen-on-the-Rhine, Germany, a firm of Germany

No Drawing. Application February 24, 1933,  
Serial No. 658,434. In Germany February 27,  
1932

6 Claims. (Cl. 260—4)

The subject matter of the invention is a process for the production of press-molding masses by condensation of phenols with formaldehyde or substances that yield formaldehyde.

- 5 Press-molding masses consisting of products of the condensation of phenols with formaldehyde have already been abundantly prepared, but the masses, that have mostly been employed, of resoles and filling agents had the disadvantage 10 that the properties of the pressed bodies were unfavorably affected by the filling agents—e. g., when using wood as filling agent, by attraction of water, and, in the case of other filling agents, by deterioration of the external condition. 15 Above all, it has been impossible to obtain glass-clear products. The employment of resoles without filling agents is impossible on account of their easy fusibility.

It is true that it has already been proposed 20 to convert the resoles by hardening more or less completely into resitols and only to press this product. No faultless results, however, have hitherto been obtained. It is true that in certain circumstances glass-clear products could be obtained, but they had considerable defects.

A press-molding mass must fulfil the following requirements:—

- (1) Great velocity of hardening,
- (2) Correctly proportioned "fluidity" which 30 depends on the one hand on the viscosity and, on the other hand, on the velocity of hardening and is determinative of the ability to be pressed, especially for the correct filling out of the molds,
- (3) Sufficient stability of shape of the finished 35 pressed piece at 160—180° C.

Now it has been found that a press-molding mass, which fulfils all these requirements, can be obtained only on observing quite definite conditions in the manufacture, which, although they 40 are partially known per se, have not hitherto been employed together in the correct manner.

In the first place, the initial material must have a definite composition. It has been recognized that only such press-molding masses are 45 usable, in which, to each molecule of phenol, a total of more than 1½, preferably 2, molecules of formaldehyde or the corresponding quantity of agents that give methylene groups and split off formaldehyde are employed. It is immaterial 50 whether, in the production of the resins, one starts with phenol and combines this with the necessary quantity of formaldehyde, or whether a resole is first prepared by combining 1 molecule of phenol with 1 molecule of formaldehyde 55 and then treating the resin with a further quan-

tity of formaldehyde, or whether novolaks are combined with hexamethylene tetramine or with the necessary quantity of formaldehyde or with both together. It is only essential that in the initial resin more than 1½, preferably 2, molecules of methylene groups are employed to 1 molecule of phenol. The basis of this requirement lies in the knowledge that only in this way can pressed bodies be obtained which when hot possess the stability of shape that is necessary 60 for the press technician, because press-molding masses which are made of formaldehyde and phenols in the proportion of less than about 1½ molecules of formaldehyde to 1 molecule of phenol and which are free from filling agents, give 65 pressed bodies which are too soft.

Even on observing the proportions stated, a usable press-molding mass could not be obtained. For this purpose, the resin must be hardened 75 to such a degree that, in the finely powdered condition, it does not sinter even at a temperature of about 70 to 100° C., but it must not become too firm because it would then not possess the necessary fluidity.

The hardening methods hitherto proposed are, 80 especially in connection with a phenoplast that hardens as rapidly as the present one such as it is essential for it to be for fulfilling the requirement 3, quite inapplicable, because the hardening cannot be retained at the suitable condition. 85

To obtain the correct hardening, the fusible resin that is obtained by condensation of the initial substances in such a proportion that more than 1½ molecules of methylene groups are employed to 1 molecule of phenol, must be 90 hardened at a moderate temperature, with supervision of the progress of the hardening or of the diminution of the fluidity, until the solidified resin gives a powder that does not sinter at about 70 to 100° C. The observation of the 95 correct temperature during the hardening is advantageously effected by filling flat molds, whose thickness should not exceed about 10 cms., with the resin and warming them in a liquid bath, preferably in a water bath, at about 100 50—70° C. In the case of thicker molds, the heat of reaction produced on hardening would not be capable of being carried away sufficiently rapidly and the resin would, at least in the middle of the mold, very rapidly become quite hard 105 and unusable. The same disadvantage would occur if higher temperatures than about 70° were chosen for the heat of the water bath. The employment of a water bath is to be preferred, because, in an air bath for example, which, 110

although it can act in a heating manner, cannot also act in a cooling manner; an undesirably rapid and uncontrollable hardening of the resin could easily occur.

- 5 With these precautionary measures, there is obtained a gradual hardening of the resin which extends over some days. In order that the limit of hardening that is favorable for the object in view shall not be exceeded, the progress of 10 the hardening must be constantly supervised. As a means for this purpose, a steel needle may be used which, loaded by a weight, penetrates more slowly into the resin as it becomes harder. The hardening of the resin is stopped as soon as the 15 velocity of the penetration of the steel needle has fallen to a certain degree that is determined by experience.

Instead of the hardening, the decrease of the fluidity can be supervised, the determination of 20 which is advantageously effected by Krahl's method (Elektrotechnische Zeitschrift, 1931, page 439).

By means of continuous supervision of the resin, one is in a position to determine exactly 25 the point of time at which the resin has reached the high melting point that is necessary for the further treatment, while maintaining a fluidity that is sufficient for the pressing. If hardening is carried on for a longer time, one would 30 be in a position to ascertain with the same method the gradually occurring deterioration of the fluidity. In this manner one has an infallible means at hand of controlling the progress of the hardening process and of protecting 35 oneself from defective results.

However, even such a resin would still be unusable for the object aimed at. The resin may, in accordance with its method of manufacture, contain water, ammonia or both, and 40 these would detrimentally affect its compressibility as well as the appearance of the pressed bodies and their usefulness. The hardened resin is consequently pulverized and the powder is then freed from water, ammonia and other volatile substances, preferably by heating at temperatures between about 80 and 100° C. and in 45 vacuo.

#### Example 1

50 A resole is prepared in a known manner from 940 parts of pure phenol, 1000 parts of 30% formaldehyde and 14 parts of hexamethylene tetramine, and a filtered solution of 230 parts of hexamethylene tetramine in 230 parts of water is then absorbed. This mixture is freed from water by vacuum distillation, the temperature gradually rising to 60° C. The mass is kept in vacuo for three more hours at this temperature.

60 The yellow resin of the consistency of honey that is obtained in this manner is now poured into metallic molds which are 60-100 cms. deep, 15-20 cms. wide and 6 up to a maximum of 10 cms. thick. The molds are suspended in a water bath at 60° C. It can be observed, on a thermometer whose mercury bulb is placed in the centre of the resin, that the temperature gradually rises to 70° C. on account of the reaction which occurs. The constantly progressing hardening is followed with an instrument which is constructed similarly to the known Vikat needle. It consists of a steel needle with a cross-sectional area of about 2 square millimetres, of which needle the bottom end is placed 70 on the resin and the top end is loaded with a

weight in a suitable manner. The resin has the correct degree of hardness when the needle, with a load of about 5 kgs., penetrates through 1 cm. in 5 to 20 minutes; this takes place in 2 to 3 days according to the quantity of water in the 80 resin.

Instead of supervising the hardness, a sample can be taken from time to time and, in the manner to be hereinafter described, converted into a powder which is free from volatile constituents and then examined as to its fluidity by the aforesaid Krahl's method. Experiments have shown that a fluidity of 100 to 200 mms. at a pressure of 300 kgs. per sq. cm. corresponds, with an accuracy that is sufficient for practical purposes, to the degree of hardness determined in the manner stated with the Vikat needle.

As soon as the resin shows the correct nature as determined in one of the manners stated, the molds with the resin are transferred from the 95 warm water baths into cold water baths. The cooled resin is converted into a fine powder and is kept for from 1 to 2 hours at a temperature of 70 to 100° C. in vacuo in a vacuum drier, so that the water and ammonia contained in the resin 100 are evaporated. A powder prepared in this manner gives, on pressing at 160° to 180° C. pressed articles which can be pushed out of the mold without becoming deformed and are yellow without further coloration and clearly transparent. 105

#### Example 2

600 parts of a novolak prepared in a known manner are mixed with a mixture of 150 parts of hexamethylene tetramine and 30 parts of wa- 110 ter at a temperature of 70 to 80° C. There is produced a resin which has the consistency of honey at this temperature and which is worked up further exactly as in Example 1.

#### Example 3

1000 parts of phenol, 1000 parts of formaldehyde and 230 parts of hexamethylene tetramine are heated for 2 hours at 60° C. It is also possible to use more formaldehyde and correspondingly less hexamethylene tetramine or vice versa. The water is then distilled off with a good vacuum and the resin is heated until it reaches a temperature of 60° C. Thereupon, the resin is kept 120 for a further 2 to 3 hours at 60° C. and is then 125 worked up further as in Example 1.

Larger quantities of formaldehyde and agents which split off formaldehyde may be employed in the examples. Instead of phenol, suitable cresols or other phenols may be employed. If desired, the temperature in the hardening may be kept somewhat lower than 50° C. or somewhat higher than 70° C., the former giving a retardation and the latter an acceleration of the 130 hardening process. Instead of the water bath there may be employed another liquid bath or, with careful working, an air bath. Instead of the Vikat needle and Krahl's method, other supervising methods for the progressing hardening may be employed. The freeing of the 135 powdered resin from volatile substances may also be effected at a lower temperature and without vacuum.

There can be added to the resin, at any desired stage during the manufacture, 1 to 5% of stearic acid and other flowing agents for the purpose of increasing the fluidity. There can also be added to the resins small quantities of 145 salicylic acid or other carboxylic acids of the 150

- aromatic series which, in a quantity of up to 10%, have the property of rendering any too large a quantity of water, which may be present in the finished products and which, in certain 5 circumstances, would produce a turbidity, harmless in this direction. Any desired quantities and kinds of organic and inorganic dyestuffs may also be added to the resins.
- Without admixture of any kind, the press-molding masses produced in the above manner, 10 give, on being worked up under pressure and heat, pressed bodies which are clearly transparent and colorless or of a yellow color.
- The above press-molding masses may be employed 15 for the production of all kinds of pressed articles for electrotechnical, household, ornamental and fancy purposes. Pressed bodies from masses according to the above process possess an excellent power of resistance to water.
- 20 I claim:—
1. A process for the production of press-molding masses by condensation of phenols with formaldehyde, comprising condensing the initial substances, in such proportions that more than 1½ molecules of methylene groups are employed to 1 molecule of phenol, into a fusible resin, 25 hardening said fusible resin in layers which do not exceed 10 centimeters in thickness at a temperature ranging from about 50° to about 70° C., 30 with supervision of the progress of the hardening until the solidified resin gives a powder that does not sinter at about 70 to 100° C., pulverizing the hardened resin, and freeing the powder from volatile substances.
  - 35 2. A process for the production of press-molding masses by condensation of phenols with formaldehyde, comprising condensing the initial substances in such proportions that more than 1½ molecules of methylene groups are employed to 1 molecule of phenol, into a fusible resin, 40 hardening said fusible resin in layers which do not exceed 10 centimeters in thickness at a temperature ranging from about 50° to about 70° C., 45 with supervision of the diminution of its fluidity, until the solidified resin gives a powder that does not sinter at about 70 to 100° C. pulverizing the hardened resin and freeing the powder from volatile substances.
  - 50 3. A process for the production of press-molding masses by condensation of phenols with formaldehyde, comprising condensing the initial substances, in such proportions that more than 1½ molecules of methylene groups are employed to 1 molecule of phenol, into a fusible resin, 55 hardening said fusible resin in layers which do not exceed 10 centimeters in thickness at a temperature ranging from about 50° to about 70° C., 60 with supervision of the progress of the hardening, until the solidified resin gives a powder that does not sinter at about 70 to 100° C., pulverizing the hardened resin, and freeing the powder from volatile substances.
- to 1 molecule of phenol, into a fusible resin, hardening said fusible resin in layers which do not exceed 10 centimeters in thickness at a temperature ranging from about 50° to about 70° C., with supervision of the progress of the hardening, until the solidified resin gives a powder that does not sinter at about 70 to 100° C., pulverizing the hardened resin, and freeing the powder from volatile substances by heating at between about 80 and 100° C. and in vacuo.
- 65 4. A process for the production of press-molding masses by condensation of phenols with formaldehyde, comprising condensing the initial substances, in such proportions that more than 1½ molecules of methylene groups are employed to 1 molecule of phenol, into a fusible resin, 70 hardening said fusible resin in layers which do not exceed 10 centimeters in thickness by heating it at about 60 to 70° C. with supervision of the progress of the hardening, until the solidified resin gives a powder that does not sinter at about 70 to 100° C., pulverizing the hardened resin, and freeing the powder from volatile substances.
  - 75 5. A process for the production of press-molding masses by condensation of phenols with formaldehyde, comprising condensing the initial substances, in such proportions that more than 1½ molecules of methylene groups are employed to 1 molecule of phenol, into a fusible resin, 80 hardening said fusible resin in layers which do not exceed 10 centimeters in thickness by heating it at about 60 to 70° C. in said form of layers not exceeding 10 cm. in thickness, in a liquid bath, with supervision of the progress of the 85 hardening, until the solidified resin gives a powder that does not sinter at about 70 to 100° C., pulverizing the hardened resin and freeing the powder from volatile substances.
  - 90 6. A process for the production of press-molding masses by condensation of phenols with formaldehyde, comprising condensing the initial substances, in such proportions that more than 1½ molecules of methylene groups are employed to 1 molecule of phenol, into a fusible resin, 95 hardening said fusible resin in layers which do not exceed 10 centimeters in thickness by heating it at about 60 to 70° C., with supervision of the diminution of its fluidity, until the solidified resin gives a powder that does not sinter at about 70 to 100° C., pulverizing the hardened resin and freeing the powder from volatile substances.
  - 100 7. A process for the production of press-molding masses by condensation of phenols with formaldehyde, comprising condensing the initial substances, in such proportions that more than 1½ molecules of methylene groups are employed to 1 molecule of phenol, into a fusible resin, 105 hardening said fusible resin in layers which do not exceed 10 centimeters in thickness by heating it at about 60 to 70° C. in said form of layers not exceeding 10 cm. in thickness, in a liquid bath, with supervision of the progress of the 110 hardening, until the solidified resin gives a powder that does not sinter at about 70 to 100° C., pulverizing the hardened resin and freeing the powder from volatile substances.
  - 115 8. A process for the production of press-molding masses by condensation of phenols with formaldehyde, comprising condensing the initial substances, in such proportions that more than 1½ molecules of methylene groups are employed to 1 molecule of phenol, into a fusible resin, 120 hardening said fusible resin in layers which do not exceed 10 centimeters in thickness by heating it at about 60 to 70° C., with supervision of the diminution of its fluidity, until the solidified resin gives a powder that does not sinter at about 70 to 100° C., pulverizing the hardened resin and freeing the powder from volatile substances.
- MAX KOEBNER.
- 139
- 125
- 140
- 145
- 150
- 55
- 60
- 65
- 70
- 75